

C. A. STETEFELDT.  
FURNACE FOR DESULFURIZING ORES.

No. 43,140.

Patented June 14, 1864.



Witnesses;

McCombs  
Henry Morris

Inventor;  
Charles A. Hobfaffer

# UNITED STATES PATENT OFFICE.

CHARLES A. STETEFELDT, OF NEW YORK, N. Y.

## IMPROVED FURNACE FOR DESULPHURIZING ORES.

Specification forming part of Letters Patent No. 43,140, dated June 14, 1864.

*To all whom it may concern:*

Be it known that I, CHARLES A. STETEFELDT, of the city, county, and State of New York, have invented a new and Improved Furnace for Desulphurizing Ores; and I do hereby declare that the following is a full, clear, and exact description thereof, which will enable any person skilled in the art to make and use the same, reference being had to the accompanying drawings, making part of this specification, in which—

Figure 1 represents a front elevation of my invention. Fig. 2 is a transverse vertical section of the same, the line  $x'x'$ , Fig. 4, indicating the plane of section. Fig. 3 is a longitudinal vertical section of the same, taken in the plane indicated by the line  $y'y'$ , Fig. 1. Fig. 4 is a plan or top view of the same. Fig. 5 is a side elevation of the same. Figs. 6, 7, and 8 are diagrams illustrating the shape and position of the terraces.

Similar letters of reference indicate the same parts in all the figures.

This invention relates to certain improvements in that class of furnaces known as "upright terrace-furnaces;" and the object of these improvements is to regulate the velocity with which the charge passes through the furnace and to reduce the time necessary for a perfect roasting or desulphurization of the ores by the peculiar shape and construction of the terraces, and by their peculiar position in relation to each other; also to reduce the expenditure of fuel and to regulate the temperature throughout the furnace by the application of hot-air apparatus and cold-air pipes in combination with the terraces, and to make such disposition in the internal arrangement that the furnace is applicable for the reduction of gold, silver, quicksilver, and other ores.

The process of roasting is undoubtedly the most important of all metallurgical operations, not only because by means of it metals are directly produced from ores and furnace products—as, for instance, in the manufacture of lead in reverberatories, the production of copper from copper matte, and the extraction of quicksilver from cinnabar—but this process also forms the basis of all other metallurgical operations.

The necessary conditions for a quick and

complete desulphurization of ores are as follows:

First. Minute division of the ores and presentation of the greatest possible surface.

Second. Introduction of the steady movement of the roasting-charge against the current of combustion gases and air. Experience shows that when the charge is left perfectly stationary, or even when it is moved with the current of air, the result is an incomplete desulphurization.

Third. Greatest possible use made of the heat generated by the process itself aside from fueling.

Fourth. A continuous and uniform mode of procedure, which renders the success of the process more independent of the attention and skill of the workmen.

My furnace is constructed with the view to fulfill these conditions. The pulverized ore is allowed to fall over a succession of terraces through an inclosed space or shaft, while a heated current of air or flame is conducted in the opposite direction. In the construction of such a furnace the form and arrangement of the terraces is the essential element, as will be apparent from the following thorough and scientific investigation. The greatest or natural slope or talus of loose masses is measured by the angle of friction,  $Q$ , inclosed by the plane of the talus and a horizontal plane. This angle will naturally be smaller when the pulverized ore, on arriving on the slope, possesses a certain initial velocity than it is when the ore is heaped thereon by careful racking from beneath. If, therefore, the angle of friction be determined by the latter method, it may be surely assumed that the ore arriving on the terraces with a certain initial velocity will slide off from the same. At the same time care must be taken to make the angle  $Q$  of the talus as small as possible, to prevent the ore from passing too quickly through the furnace. By various experiments with different crushed ores the angle of friction for careful piling was found to be about thirty-five degrees. The slope of the terrace measured by the angle  $B A D$ , Fig. 6, therefore, is to be thirty-five degrees, and consequently the angle  $A B D$  inclosed by the two sloping sides of terrace will be one hundred and ten degrees.

In order to determine the position of the





It is unnecessary to continue the calculation any further, since the values of  $H$  will be alternately 0.5663 feet and 0.7644 feet. The velocity of the ore will therefore become zero after passing two terraces, and a periodical or intermittent motion will be the result, which is of the greatest importance for the success of the roasting process.

By the aid of the equations 6 and 8, and by using the values of  $C_{II}$ ,  $(H_2 - h)$ ,  $C_s$ ,  $C_{III}$ , and  $(H_3 - h)$  as determined by the above example, we find the value of  $T$ , the time of one period:  $T = 0.2299 + 0.1136 + 0.1976 + 0.0631 = 0.6042$  seconds; and since each period covers two terraces, it follows that if the furnace contains twenty terraces the ore will remain in it 6.042 seconds.

The quantity of ore which may be thrown upon the uppermost terrace is limited by the velocity of the current of air in the sections of the furnace. This velocity ought to exceed five feet per second, and taking the following dimensions as a basis, we can find the quantity of the charge: Let the length of the terrace be three feet,  $h$ ,  $2b$ , &c., the same as above stated, and the charge consists of iron pyrites, which are to be deprived of their entire contents of sulphur—viz., 53 per cent. We assume that 25 per cent. of the oxygen does not take part in the roasting, but escapes unchanged. The temperature in the furnace shall not exceed  $700^{\circ}$  centigrade, ( $1,223^{\circ}$  Fahrenheit.) Three English feet being 0.916 meters, there will pass through the section of one feeder in one second 340,840 cubic centimeters of air heated to  $700^{\circ}$  centigrade. At a temperature of  $0^{\circ}$  centigrade, and the barometer at 0.76 meter, (30 inch,) this air would take up a space of 95,594 cubic centimeters, weighing 123.6 grams; but of this quantity 21.01 grams of oxygen act in the process and unite with 21.01 grams of sulphur to sulphurous acid, (50.) This result corresponds to 39.65 grams of pyrites per second, which will give for twelve hours 1,713,000 grams, or 34.26 hundred-weight @ one hundred pounds @ five hundred grams to the pound. For a furnace with five feeders, the product of twelve hours will be one hundred and seventy-one hundred-weight. Pulverized ores contain about one-third of their volume in empty interstices, and since the specific gravity of pyrites is 5, the 39.65 grams of ore required per second will take up a space of 11.9 cubic centimeters, which the feed-rollers must supply. If the latter are supplied with semicircular flutes, it will be easy to calculate the number of revolutions required per minute.

Guided by the results obtained by this investigation I built my furnace in the following manner:

K represents an upright shaft of rectangular section built up of brick and lined with fire-brick or any other suitable material. This shaft contains the terraces L, which are diamond-shaped, as clearly shown in Fig. 2 of the drawings, so that they can be turned if the

upper side has been injured, and thus will be more durable and absorb and recommunicate more heat than they will if made with a triangular cross-section. They must be made of fire-clay and had better be covered with a coating of graphitic clay, which resists most perfectly the chemical action of the roasting-charge. A square iron rod is placed in the center of each terrace, so that the same can be built in the rear and front wall of the furnace. The roof N of the furnace which is formed of fire-clay contains the feed-openings F, and above these are situated the rollers E, by which the ore can be conveyed regularly and in the desired quantities to the furnace. These rollers may be fluted in a direction parallel to their axis. From the rollers the ore drops upon a roof-shaped surface, e, which checks its velocity. The sides of this roof are perpendicular to the slope of the sides of the feed-openings. On both sides of the shaft K are the fire-places G, which serve for heating up the furnace, and in certain cases for keeping up a fire during the process of roasting. The fire-places and ash-holes are so arranged that a draft can be created from beneath through the pipes a'. After the ore has passed down over the terraces L, it collects in the lower part of the shaft and can be removed through an aperture, b', and a subterranean passage, d'. When blonde is roasted, it may be advisable to prolong the lower end of the furnace into a hearth. Above the arch of the fire-place in each side of the furnace a pipe, d, is set, which conveys the heated air from the bellows. This pipe may set lower down into the furnace below the fire-places on the sides of the pipes a', in which case the number of terraces may be increased by putting an additional number below the level of the fire-bridge. Between this level and that of the arch of the fire-place no terraces should be put, since they would prevent the uniform distribution of the flame in the furnace.

While building the front wall of the furnace, holes f' should be left opposite each terrace, so that the temperature in the shaft may be observed and disturbances may be remedied by means of proper tools. During the roasting these openings must be closed.

Behind the shaft K is a chamber, K', Fig. 3, which contains a series of oval pipes, g'. These pipes communicate with the bellows, and through them the air for the bellows is heated. The shaft K communicates with the chamber K' by means of a flue, h', which is partially occupied by the uppermost terraces. On leaving the chamber K' the gases pass into the channel I, which leads to the chimney J, and above this channel the wet ores from the stamps are spread to be thoroughly dried.

This furnace is applicable to the desulphurization of ores of every description, but particularly for treating auriferous sulphurets and metals which are afterward to be treated by amalgamation. For materials rich in sulphur no fire will be required after the furnace

has once been heated. It will then run itself, heating its own air, and requiring only to be kept charged. Zinc blende can be desulphurized with very little fire. When it is desired to desulphurize ores and furnace products only to a certain degree, (which is the case in most smelting operations,) the process can be perfectly regulated by the amount of ore conducted through the feeders, the quantity of air admitted, and the height given to the furnace.

For many purposes, especially for roasting auriferous sulphurets, the bellows can be entirely dispensed with, and a chimney with a strong draft substituted.

I am aware that a mode of roasting analogous to mine in its general principles is described in a patent granted to Keith, Behr, and Keith on the 9th of September, 1862; but my process is superior to theirs, by reason of the use of hot-air blast and the means afforded for applying a greater amount of heat to the ore within a given height of shaft.

I am also aware that the general idea ofter-

races is not new, and that a roasting-shaft is described by Whelpley and Storer in their patent of January 12, 1864.

What I claim as new, and desire to secure by Letters Patent, is—

1. The employment or use of an upright terrace-furnace, substantially such as herein described, for the purpose of reducing gold, silver, quicksilver, and other metals from the sulphureted ores.

2. The peculiar construction, proportion, and disposition of the terraces L in the shaft K, as based on the rules deduced from the formulæ 1 to 24, whereby a complete and rapid desulphurization of the ores is accomplished.

3. The combination of a hot-air apparatus with an upright terrace-furnace, for the purpose substantially as set forth.

CHARLES A. STETEFELDT.

Witnesses:

W. HAUFF,

M. M. LIVINGSTON.